

Sept. 25, 1934.

A. VON BIEHLER  
PHOTOGRAPHIC MATERIAL  
Filed March 8, 1932

1,974,524

*Fig. 1*



*Fig. 2*



*Fig. 3*



*Inventor:*

*Arpad von Biehler,  
By Attorney  
Philip S. Hopkins.*

## UNITED STATES PATENT OFFICE

1,974,524

## PHOTOGRAPHIC MATERIAL

Arpad von Biehler, Dessau in Anhalt, Germany,  
assignor to Agfa Ansco Corporation, Binghamton, N. Y., a corporation of New York

Application March 8, 1932, Serial No. 597,639  
In Germany March 9, 1931

8 Claims. (Cl. 95—81.5)

My present invention relates to photographic filter layers.

Filter layers for photographic purposes which are, for instance, required in the multi-pack processes of the color photography, are prepared with dyestuffs which diffuse as little as possible, especially if such layers are superposed. The dyestuffs hitherto described, however, are soluble in water and show an appreciable diffusion when incorporated in thick, relatively slow drying layers.

I have found that any troublesome diffusion is avoided by finely dispersing a water-insoluble dyestuff in a binding agent forming the base of the filter layer. Such binding agents are gelatin, glue, agar-agar and the like water-soluble colloids. When the binding agent has been sufficiently mixed with the insoluble dyestuff, filter layers can be prepared which, after drying, are completely homogeneous and transparent. The mixing is effected with mechanical means in apparatus well known to those skilled in the art.

Suitable organic pigments are all of the water-insoluble organic color lakes which do not detrimentally influence the light-sensitive photographic layers. I prefer the earth alkali metal salts, such as the barium or calcium salt and the heavy metal salts, such as the bismuth or especially the lead salt of acid dyestuffs which are liable to be decolorized in a suitable manner without the silver picture of the photographic material being injured. As dyes suited for the purpose set forth I enumerate among others the Sirius dyes, Benzolichtgelb (cf. Fierz-David, "Künstliche organische Farbstoffe" 1926, page 168), Congo red and Congo blue. The color lakes are prepared according to the methods well known in the art of dyeing with the difference that the precipitation is effected in the absence of a substratum.

The precipitated color lakes are in the form of a paste or pulp, intimately mixed with the binding agent until a homogeneously colored mass is formed. The filter layer can be arranged in, before or behind the light-sensitive emulsion layer. In the first case the light sensitive emulsion is mixed with the color particles. The layer thus produced can be employed for the production of color pictures made according to one of the direct processes. In the second case the colored layer acts as a light filter and is adapted to select light of a certain wave length for the exposure. In the third case, if the filter layer is arranged behind the light sensitive emulsion layer the former acts as an anti-halation layer. I prefer, however, to apply my filter layers in front

of the light sensitive emulsion layer or behind the same.

In the accompanying drawing Figs. 1 to 3 show the aforesaid arrangements.

In Fig. 1 the filter layer consisting of a binding agent and a color lake is provided on the photographic film consisting of a support and a light sensitive emulsion layer.

In Fig. 2 the color lake is distributed in the emulsion layer which is provided on the usual support.

In Fig. 3 the filter layer consisting of a binding agent and a color lake is arranged between the emulsion layer and the support.

The following example illustrates the invention:

An aqueous solution of Congo red is mixed with an aqueous solution of barium chloride until a precipitate is no longer formed. The precipitate is purified by decanting and then mixed with an aqueous gelatin solution of 10 per cent strength having a temperature of 40° C. The whole is intimately mixed until it assumes the appearance of a uniformly colored, transparent mass. The filter layers are then prepared in the usual manner by casting. The dyestuff-gelatin layer thus formed is transparent and does not show any diffusion even in a wet state. By bathing it in an acidified solution of sodium hydrosulphite it can be easily decolorized.

My invention is not limited to the foregoing example nor to the specific details given therein. The quantity of dyestuff to be added to the solution of binding agent is dependent upon each special purpose and can be determined by a few simple experiments. Other color lakes than those mentioned can be used with success. I contemplate as being within the spirit of my invention all such modifications as fall within the scope of the appended claims.

What I claim is:

1. A photographic filter layer which comprises a color lake of an acid azo dyestuff, and a binding agent.
2. A photographic filter layer which comprises an earth alkali metal salt of an acid azo dyestuff removable without injuring a photographic silver picture and a binding agent.
3. A photographic filter layer which comprises a heavy metal salt of an acid azo dyestuff removable without injuring a photographic silver picture and a binding agent.
4. A photographic filter layer which comprises the lead salt of a Sirius dye and a binding agent.

5. A photographic filter layer which comprises the barium salt of Congo red and gelatin.
6. The process of producing photographic filter layer which comprises precipitating from a solution of an acid azo-dyestuff the dyestuff in form of a color lake, purifying the precipitate, mixing the precipitate with the solution of a binding agent, and casting a filter layer from the said mixture.
- 15 7. The process of producing photographic filter layer which comprises precipitating from a solution of an acid azo-dyestuff the dyestuff by means of a compound selected from the group consisting of earth alkali metal salts and heavy metal salts, purifying the precipitate, mixing the precipitate with the solution of a binding agent, and casting a filter layer from the said mixture.
8. The process of producing photographic filter layer which comprises precipitating from a solution of Congo-red the dyestuff by means of barium-chloride, purifying the precipitate, mixing the precipitate with an aqueous solution of gelatin, and casting the filter layer from the said mixture.

ARPAD v. BIEHLER.

|    |     |
|----|-----|
| 15 | 90  |
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |